

# United States Patent Office

3,288,689

Patented Nov. 29, 1966

1

3,288,689

## METHOD FOR COATING METAL OBJECTS WITH ALUMINUM

Kuninori Azuma, Nara-ken, Japan, assignor to Matsushita Electric Industrial Co., Ltd., Osaka, Japan, a corporation of Japan

No Drawing. Filed Feb. 27, 1963, Ser. No. 261,528

Claims priority, application Japan, Mar. 1, 1962, 37/8,063; Nov. 12, 1962, 37/51,160

5 Claims. (Cl. 204—29)

This invention relates to a method for coating metal with aluminum by use of anhydrous fused salt, and more particularly to an improved method involving electroplating with aluminum by use of anhydrous fused salt wherein the objects to be plated, e.g. steel band or steel wire are passed through a bath containing water-soluble additives and dried before electroplating.

It is known to plate aluminum on various metal objects, e.g. steel wire from an anhydrous fused salt electrolyte; namely, the double salt of aluminum chloride and alkali metal chloride. It is also known to add alkali metal halide e.g. sodium fluoride or potassium fluoride as an additive and fuse together.

Prior to this application the inventor filed U.S. patent application Serial Number 195,422, now Patent No. 3,236,751, in which he provided an anhydrous fused salt electrolyte, namely, the double salt of aluminum chloride and alkaline earth metal chloride e.g. barium chloride or strontium chloride and, as an additive, alkali metal borofluoride e.g. sodium borofluoride or potassium borofluoride.

The most difficult problem of electroplating of aluminum by the anhydrous fused salt method is that of metal fog formed on the aluminum anode by an increase of bath temperature of the fused salt and current density.

When this fog appears while plating, it adversely affects current efficiency and liberated fine particles of aluminum grow into wood-branch-like crystal on the plating surface which prevents the coating from growing thicker, or liberated fine particles of aluminum become sponge-like floatings which adhere on the plating surface, spoil it and become an origin of corrosion.

Furthermore, when electroplating with the fused salt is continued, partial consumption of electrolyte components by evaporation which is inevitable in keeping the fused salt at the temperature about 160° C., or aging of electrolyte components are induced, and thereby current density suddenly decreases and becomes a cause of bad plating.

These defects have been a serious obstacle in the continuous plating on a commercial scale of e.g. steel band and the like.

The present invention provides a method in which a bath containing water-soluble salt is arranged before the electroplating bath and by which the obstacle to continuous plating operation i.e. aging of electrolyte bath is removed and the production of beautiful, anticorrosive plating of aluminum is thereby possible.

Though the method of this invention is not restricted by the composition of the electroplating bath, the following are suitable compositions by weight which serve the purpose.

(a)

Percent

Aluminum chloride ----- 60 to 85  
Alkaline earth metal chloride ----- 10 to 25  
Alkali metal borofluoride ----- Less than 0.5

or

(b)

Percent

Aluminum chloride ----- 60 to 85  
Sodium chloride ----- 10 to 20  
Alkaline earth metal chloride ----- 10 to 35  
Alkaline earth metal fluoride ----- 0.3 to 5

2

or

Aluminum fluoride ----- 0.5 to 10

The water-soluble additive in the bath is composed of aluminum chloride and either alkaline earth metal chloride or alkali metal chloride and metal fluoride, and a composition which is effective for the purpose is as follows wherein percentages are by weight.

10

(c)

Percent

Aluminum chloride ----- 10 to 25  
Alkaline earth metal chloride or alkali metal chloride ----- 0.1 to 10  
15 Alkaline earth metal fluoride or metal fluoride ----- 0.1 to 5

Among the above compositions, that are shown hereunder is preferable for the water-soluble additive.

20

(d)

Percent

Aluminum chloride ----- 10 to 20  
Alkaline earth metal chloride ----- 0.5 to 10  
25 Alkaline earth metal fluoride ----- 0.5 to 2

or

Aluminum fluoride ----- 0.5 to 5

30

When the water-soluble additive of the (d) composition is used, a plating bath of the (b) composition is effective.

35

As for the temperature of the bath containing the water-soluble additive, ordinary room temperature is employed, however, in order to effect the drying process in the successive step smoothly, a temperature slightly higher than room temperature is favored. If the temperature is too high, metallic compounds existing in the water-soluble additives are converted into oxides, which is undesirable.

40

The preferred range is between room temperature and 80° C. When the temperature of the process is low, drying cannot be conducted sufficiently, and when the temperature is too high, aluminum chloride is vaporized, causing the formation of metallic oxides. Therefore, a temperature of 200±10° C. is preferable.

45

As an alkaline earth metal of the plating bath, barium is preferable, because its potential becomes considerably more basic, sometimes more basic than that of alkali metal. Further, when the electroplating is conducted with a bath containing alkaline earth metal chlo-

50

ride and fluoride, appearance of metal fog is much more greatly reduced than with any other fused salt plating bath of the same temperature and using the same current density. Current efficiency is high, the plating surface is beautiful, coating is thick and the anti-corrosive property

55

is excellent. It is easy to obtain a coating having a thickness of 7μ to 13μ. Moreover, it is possible to make the current density greater than that obtained by any other electrolyte, and accordingly it is possible to increase the line speed of continuous plating of e.g. band steel and boost up production efficiency.

60

The melting point of the plating bath varies according to the proportion of each component, but generally it is about 110° C. Though it is preferable to make the plating temperature as low as possible, it is difficult to obtain a bright plating surface at a temperature below 140° C. because of low plating efficiency, and at a temperature higher than 175° C. formation of metal fog is increased. Therefore, a plating temperature of 160±5° C. is most suitable.

70

The following examples are given to show the embodiments of this invention.

*Example I*

As an electroplating bath, the following composition is used.

|                     | Percent |
|---------------------|---------|
| Aluminum chloride   | 78      |
| Barium chloride     | 13      |
| Strontium chloride  | 8.6     |
| Sodium borofluoride | 0.4     |

Also as a water-soluble additive bath the composition as shown hereunder is used.

|                   | Percent  |
|-------------------|----------|
| Aluminum chloride | 10 to 25 |
| Aluminum fluoride | 0.1 to 1 |
| Lead fluoride     | 0.1 to 1 |
| Barium chloride   | 0.1 to 1 |

*Example II*

An electroplating bath having the following composition is used.

|                        | Percent |
|------------------------|---------|
| Aluminum chloride      | 75      |
| Sodium chloride        | 10      |
| Barium chloride        | 8       |
| Strontium chloride     | 6.6     |
| Potassium borofluoride | 0.2     |
| Lithium chloride       | 0.2     |

Also a water-soluble additive bath composition is used.

|                   | Percent  |
|-------------------|----------|
| Aluminum chloride | 10 to 25 |
| Aluminum fluoride | 0.1 to 1 |
| Lead chloride     | 0.1 to 1 |
| Lithium chloride  | 0.1 to 1 |

*Example III*

An electroplating bath having the following composition is used.

|                   | Percent |
|-------------------|---------|
| Aluminum chloride | 70      |
| Sodium chloride   | 15      |
| Barium chloride   | 11      |
| Aluminum fluoride | 4       |

A water-soluble additive bath having the following composition is used.

|                                | Percent |
|--------------------------------|---------|
| Aluminum chloride              | 10      |
| Barium chloride                | 5       |
| Aluminum fluoride <sup>1</sup> | 3       |

<sup>1</sup> Aluminum fluoride is used after converting it into the hydrate of aluminum fluoride  $\text{AlF}_3 \cdot 3\frac{1}{2}\text{H}_2\text{O}$ .

*Example IV*

An electroplating bath having the following composition is used.

|                   | Percent |
|-------------------|---------|
| Aluminum chloride | 70      |
| Sodium chloride   | 15      |
| Barium chloride   | 12      |
| Barium fluoride   | 3       |

A water-soluble additive bath having the following composition is used.

|                   | Percent |
|-------------------|---------|
| Aluminum chloride | 10      |
| Barium chloride   | 5       |
| Barium fluoride   | 4       |

In each example steel band was passed through a room temperature solution of a water-soluble additive bath and

dried at 200° C. to deposit the water-soluble additive on the surface of the steel band. Next the steel band was immersed, as a cathode, in an anhydrous fused salt electrolyte bath at the temperature of 160° C., against an anode of pure aluminum, D.C. current was passed at the density current of 3 a./dm.<sup>2</sup>. After 5 minutes of plating, 6μ and after 10 minutes 10μ of aluminum coating were obtained. In each case the plated coating was smooth and very lustrous. Its adherence was excellent and current efficiency was high, and continuous operation was possible.

In summary, this invention provided an improved method of continuous electroplating of aluminum by the anhydrous fused salt method which is characterized in dipping the object to be plated in a bath of water-soluble additive consisting essentially of aluminum chloride before dipping in the anhydrous fused salt plating bath, drying the above object, whereby the water-soluble additive deposits on the surface and then dipping the same object in the anhydrous fused salt plating bath. This method affords a beautiful aluminum coating continuously and is very valuable in commercial practice.

What is claimed is:

1. In the method for coating ferrous objects with aluminum using the anhydrous fused salt electroplating process, the improvement consisting first of immersing the object to be plated in an aqueous solution of water-soluble additives consisting of aluminum chloride, at least one chloride selected from the group consisting of alkali metal chloride and alkaline earth metal chloride and at least one fluoride selected from the group consisting of alkaline earth metal fluoride, aluminum fluoride and lead fluoride, said water-soluble additives consisting essentially of about 10% to 25% of aluminum chloride, about 0.1% to 10% of at least one chloride selected from the group consisting of alkaline earth metal chloride and alkali metal chloride and about 0.1% to 5% of at least one fluoride selected from the group consisting of alkaline earth metal fluoride, aluminum fluoride and lead fluoride, then drying the object whereby the surface is coated with the additives of said aqueous solution and then introducing the object into the electroplating bath.

2. Method according to claim 1 wherein the temperature of the aqueous solution ranges from room temperature to 80° C.

3. Method according to claim 1 wherein the object is dried at a temperature of 190-210° C. after immersion in the aqueous solution.

4. Method according to claim 1 wherein the additives consist by weight of 10% to 20% aluminum chloride, 0.5 to 10% of alkaline earth metal chloride and 0.5% to 2% of alkaline earth metal fluoride.

5. Method according to claim 1 wherein the water-soluble additives consist by weight of 10% to 20% of aluminum chloride, 0.5% to 10% of alkaline earth metal chloride, 0.5% to 5% of aluminum fluoride.

**References Cited by the Examiner****UNITED STATES PATENTS**

|           |         |               |          |
|-----------|---------|---------------|----------|
| 2,315,725 | 4/1943  | Moller        | 117-114  |
| 2,709,154 | 5/1955  | Hansgirg      | 204-39   |
| 2,971,899 | 2/1961  | Hanink et al. | 204-29   |
| 3,007,854 | 11/1961 | Smith et al.  | 204-39 X |
| 3,048,497 | 8/1962  | Moller        | 204-39 X |

JOHN W. MACK, Primary Examiner.

G. KAPLAN, Assistant Examiner.